

Nov. 5, 1957

W. O. YOUNG, JR

2,811,770

PREPARATION OF TOW FROM FILAMENTS OF ACRYLONITRILE POLYMERS

Filed Dec. 8, 1953

*Fig. 1.*



*Fig. 2.*



INVENTOR  
*William Oliver Young Jr.*

BY *C. H. Mortenson*

ATTORNEY

# United States Patent Office

2,811,770

Patented Nov. 5, 1957

1

2,811,770

## PREPARATION OF TOW FROM FILAMENTS OF ACRYLONITRILE POLYMERS

William Oliver Young, Jr., Camden, S. C., assignor to E. I. du Pont de Nemours and Company, Wilmington, Del., a corporation of Delaware

Application December 8, 1953, Serial No. 396,978

2 Claims. (Cl. 28—78)

This invention relates to an improved guiding arrangement for bringing together a plurality of filament bundles to form a larger composite bundle or tow.

In the manufacture of staple and tow of continuous crimped filaments, such as those of polyacrylonitrile and copolymers of acrylonitrile containing not less than 85% acrylonitrile, the filament bundles from each spinning machine or from a group of spinning machines are washed and drawn and then, before being subjected to crimping and/or drying, several moist ribbons of filaments are combined to form a very large denier tow. Heretofore, the several smaller bundles after passing through a pin or comb guide were brought together over a bar guide where the individual bundles flattened out and widened perceptibly so that they continued on as a single wide ribbon to the crimper. This combined tow of crimped filaments tended to split when subjected to cutting or during drying prior to their sale as a continuous filament tow, and in the customers' mills the tow of continuous crimped filaments caused trouble by splitting into the several smaller bundles. Tow which splits in any of the processing steps causes excessive "downtime" and waste due to tangling; costs increase and the quality of the final product is lowered.

It is, therefore, an object of this invention to provide an improved process for overcoming this defect. Another object of this invention is to prepare a tow of continuous filaments comprised of a plurality of smaller tows that have been overlapped so as to resist splitting. Still another object of this invention is to provide an improved guiding arrangement for producing an overlapped tow. Other objects will be apparent from the description of the invention that follows.

The objects of this invention are accomplished by means of guide bars placed substantially parallel and spaced several inches apart. The several individual moist ribbons of filaments, which have been washed and drawn and kept segregated during these processing steps, are delivered, usually through a pin or comb guide, to the first of the bar guides. As can be observed from Figure I, the ribbons are brought over the first bar guide by passing alternate preliminary tows over and under the first bar guide and then all go over the second guide. The individual elemental tows spread during and after contact with the bar and since there is no interference with adjacent tows, a certain amount of overlapping results by the time all of them pass over the second guide bar. It is this overlapping of the preliminary tows that effectively binds the final tow into a unitary bundle that very greatly improves subsequent processing or conversion into a finished product.

In previous handling the individual ribbons were passed over the first bar and over the second as one wide ribbon. In this arrangement there was, of course, contact of a ribbon with the edges of its adjacent ribbons, but this contact was insufficient to prevent the adverse splitting. In the present handling, there is overlapping and a well-bound tow results.

2

Figure I shows the arrangement of the guide and tow and Figure II shows, in an end view, the nature of the overlap.

In Figure I guide bar 1 and guide bar 2 are located in a substantially parallel arrangement. A plurality of moist ribbons 3 come from a source to guide bar 1 and here they are passed alternately over and under guide bar or cylinder 1. For example, ribbons 4 and 5 are shown going under guide bar 1, while ribbons 6 and 7 are shown going over. Each ribbon is, of course, made up of a plurality of filaments 8. They are joined as they go over bar 2 and the overlaps 9 result so that the final product is a unitary tow 10 comprised of a plurality of individual tows adjacently overlapped with each other. 15 This overlap 9 need not be extensive and is generally of a small magnitude, being about 20% of the total width of the single ribbons, although the overlap may vary from about 10% to about 40%.

In Figure II it can be seen that the individual filaments 8 are retained substantially in their respective ribbons and that the overlap is formed chiefly by the contact of a portion of the bottom of one ribbon with a portion of the top of another, adjacent ribbon. The extent of the overlap is designated at A in Figure II. There may be some intermingling or intermeshing of filaments from the different contacting tows but generally the amount of such positioning is very small. With the contact as shown very good binding occurs with many types of filaments such as those prepared from polyacrylonitriles, polyesters, polyamides and cellulose materials.

The guiding means are preferably cylindrical although other shapes, such as substantially rectangular or oval shapes can be used. They are made preferably of stainless steel or other non-corrodible, wear-resistant materials. Plastic, glass and ceramic materials may also be used. Other means may be devised for producing an overlapped tow as above described and combinations of crowned rolls or bent bars may produce even greater spreading and overlapping of tows which may be desirable under certain conditions.

The following example is given to illustrate the surprising improvement in running continuity and quality of the resulting crimped tow for sale to converters.

Over a given unit of time production was followed for off-quality material and for operating efficiency, using 45 the normal non-overlap producing procedure. In this test, 31.1% of the production was not first-quality and operating efficiency was only 57%. In other tests using the principles of this invention, the off-quality material was reduced considerably to a low level of about 7% and operating efficiency, measured on a relative basis, was increased to 100%. These results are shown in the table below:

|                    | Percent Off-Quality | Percent Operating Efficiency |
|--------------------|---------------------|------------------------------|
| Old Guide.....     | 31.1<br>7.4         | 57<br>62                     |
| Overlap Guide..... | 7.7<br>6.5          | 92<br>100                    |

Another advantage provided by this invention is that the amount of first grade material produced in a unit time can be substantially increased, since the operation is 65 more efficient and less downtime is experienced. The very substantial improvement in quality and the much improved continuity of operation lowered costs of production. Furthermore, mill converters of this improved or overlapped crimped filament tow report their operating 70 efficiencies are substantially increased and in one case nearly doubled.

It is indeed surprising that the simple expedient above described consolidates the elemental filament bundles and provides sufficient cohesion through the slight overlap to keep the resulting tow intact during subsequent operations. This overlapped tow is crimped in a "stuffer box" type crimper such as described in Hitt U. S. Patent 2,311,174 more uniformly and with noticeable improved efficiency. The crimped overlapped tow is cut into staple more effectively, that is, the "downtime" and waste are reduced. The overlapped tow of crimped continuous filaments sold as such to converters is of improved quality as is evidenced by improved efficiency in converting this tow to top due to reduction in tow splitting and breaks in the tow.

Any departure from the above description which conforms to the present invention is intended to be included within the scope of the claims. 15

I claim:

1. A composite tow comprising a plurality of tow

ribbons consisting substantially of parallel longitudinally disposed continuous filaments of a polymer of acrylonitrile, each of said tow ribbons overlapping its adjacent ribbon from 10% to 40% of its width in lightly bound relationship.

5 2. The tow of claim 1 in which the overlap is about 20%.

References Cited in the file of this patent

10 UNITED STATES PATENTS

|           |              |                |
|-----------|--------------|----------------|
| 2,055,412 | Hurst et al. | Sept. 22, 1936 |
| 2,181,777 | Asbelle      | Nov. 28, 1939  |
| 2,369,395 | Heymann      | Feb. 13, 1945  |
| 2,475,052 | Rosen        | July 5, 1949   |
| 2,494,965 | Rosen        | Jan. 17, 1950  |
| 2,677,007 | Jensen       | Apr. 27, 1954  |